

# UNITED STATES PATENT OFFICE.

YNOCENCIO GONZALEZ-GOMEZ, OF CASCANTE, NAVARRE, SPAIN.

## MATCH AND MODE OF MAKING.

### SPECIFICATION forming part of Letters Patent No. 426,007, dated April 22, 1890.

Application filed October 8, 1889. Serial No. 326,338. (No model.) Patented in Spain April 12, 1889, No. 9,370, and in England September 11, 1889, No. 14,362.

*To all whom it may concern:*

Be it known that I, YNOCENCIO GONZALEZ-GOMEZ, a subject of the King of Spain, and a resident of Cascante, Navarre, Spain, have 5 invented certain Improvements in the Manufacture of Matches, (for which patents have been granted in Spain, No. 9,370, dated April 12, 1889, and in Great Britain, No. 14,362, dated September 11, 1889,) of which the following is 10 a specification.

My invention relates to what are known as "wax matches," and particularly to that class of such matches wherein the wax impregnates or covers a core or stick of stiff card-board or 15 paper.

The object of my invention is to produce a more finished and perfect match than those of this class made in the usual manner.

In carrying out my invention I take stiff 20 card-board or bristol-board, or even heavy paper, and cut it into narrow strips by means of a suitable cutter—as a guillotine-press, for example. The width of the strips will depend on the thickness and strength of the material 25 from which they are cut, and also upon the size and strength which the bodies of the matches are desired to possess. The strips are then placed in a cutting-frame and cut to the desired length to form the stick of the 30 match, or they may be so cut by hand. The sticks so cut or the strips or widths before cutting are then immersed for a proper length of time in a bath composed of four kilograms of colophony and one kilogram of stearine, to 35 which may be added a suitable proportion of coloring-matter if the sticks are desired to be colored. After drying, the matches are passed through a draw-plate or between rolls, which compacts the coating and gives to the matches 40 a smooth, finished, and rounded form. They are then dipped in an ignitable compound, as phosphorus composition, to provide them with the ordinary igniting tips or heads. The

drawing or rolling may be done before or after the strips are cut into lengths for the matches. 45

Matches prepared by my improved process are of a very neat appearance and are capable of being burned throughout their whole length after ignition at the tip and are susceptible of even a higher finish than can be 50 given to the ordinary wax match.

Having thus described my invention, I claim—

1. As an improved article of manufacture, a match having a stick of card-board or heavy 55 paper covered and impregnated with an inflammable composition of the character described, pressed into a rounded or other finished shape, and having a tip or head of phosphorus or other ignitable composition, sub- 60 substantially as set forth.

2. The improved process of making matches, which consists in first cutting the stick or body of the match from a sheet or strip of card-board, heavy paper, or the like, then impregnating or covering the same with an inflammable composition, then drying the same, and then pressing the same into a round or other finished form, substantially as set forth. 65

3. The improved process of making matches, 70 which consists in first cutting the stick or body of the match from a sheet or strip of card-board, heavy paper, or the like, then impregnating or covering the same with an inflammable composition, then drying and pressing 75 the same into a rounded or other finished form, and then tipping the same with ignitable material, substantially as set forth.

In witness whereof I have hereunto signed my name in the presence of two subscribing 80 witnesses.

YNOCENCIO GONZALEZ-GOMEZ.

Witnesses:

MARTIN GONZALEZ,  
ALFRED FERNANDEZ.